

## UNITED STATES PATENT OFFICE

2,427,272

## MINERAL OIL COMPOSITION

Everett W. Fuller, Woodbury, N. J.; Horace E. Redman, Wyandotte, Mich., and Henry G. Berger, Glen Rock, N. J., assignors to Socony-Vacuum Oil Company, Incorporated, a corporation of New York

No Drawing. Application May 18, 1944,  
Serial No. 536,196

13 Claims. (Cl. 252—32.7)

1

This invention has to do with the stabilization of petroleum products against the harmful effects of oxidation and deterioration with use. More specifically, it has to do with the improvement or stabilization of mineral oil fractions, particularly viscous mineral oils, by the use of novel reaction products, or a novel class of reaction products, which when admixed with a mineral oil in minor proportions will prevent or delay undesirable changes taking place in the oil.

To those familiar with the art it is well known that substantially all of the various fractions obtained from mineral oils and refined for their various uses are susceptible to oxidation. This susceptibility of an oil fraction to oxidation and the manner in which oxidation manifests itself within the oil varies with the type and degree of refinement to which the oil has been subjected and with the conditions under which the oil is used or tested. In other words, the products formed in an oil fraction as a result of oxidation and the degree to which they are formed depends upon the extent to which the various unstable constituents which may act as oxidation catalysts have been removed by refining operations and also upon the conditions of use.

A large number of characterizing ingredients have been proposed for use as improving agents for petroleum products. For example, various materials containing sulfur or phosphorus, or combinations of these elements, have been suggested as stabilizing agents for viscous petroleum oils. Phosphorus- and sulfur-containing reaction products of numerous hydrocarbons and  $P_2S$ s are typical examples of such agents. Although some of these reaction products are fairly effective as mineral oil stabilizing agents, many of them are not entirely satisfactory for various reasons. Some considerably darken the oils in which they are incorporated, thereby militating against their use. Others suffer also from the disadvantage of limited oil solubility and sludge-like character. Still others are undesirable in the relatively small amounts of sulfur and phosphorus present therein. All of the foregoing undesirable characteristics seriously reduce the saleability of such products in the oil industry.

The present invention is predicated upon the discovery of a novel class of oil-soluble, acidic, phosphorus- and sulfur-containing reaction products, and the ammonium and metal salts thereof, which are capable of effecting improvement of petroleum fractions, particularly viscous mineral oil fractions. These reaction products, and the said salts thereof, prevent the for-

2

mation of acidic oxidation products and sludge in an oil, as well as inhibit the corrosion of metal engine parts such as alloy-metal bearings which come in contact with the oil. The said improving agents are particularly desirable in view of the following features: they do not impair the color of the oil fraction in which they are incorporated; they contain substantial quantities of phosphorus and sulfur; they do not contain sludge-like constituents, and they are readily soluble in oil fractions.

The improving agents contemplated herein are oil-soluble, acidic, phosphorus- and sulfur-containing reaction products obtained by reaction of phosphorus pentasulfide and an oxidized paraffin wax at an elevated temperature between about 50° C. and about 125° C., and particularly at about 100° C. As indicated hereinabove, the ammonium and metal salts of the aforesaid reaction products are also contemplated.

The oxidized paraffin wax reactants used in preparing the aforesaid improving agents are obtained by the oxidation of paraffin wax, or paraffin slackwax which contains a predominant proportion of paraffin wax, in combination with an oil fraction. The paraffin slackwaxes contemplated herein should contain at least about 75 per cent of paraffin wax, in order to obtain effective and desirable reaction products of the type defined above. The paraffin waxes generally contain at least about 18 carbon atoms, although a paraffin wax containing on the average of about 24 carbon atoms and having a melting point of about 126° F. is preferred. As used herein, and in the appended claims, the term "paraffin wax" is inclusive of the slackwaxes described above. To oxidize these waxes, air or oxygen is introduced into a quantity of wax at an elevated temperature of the order of from about 120° C. to about 180° C., and preferably at about 160° C. Temperatures below 120° C. may also be used in the oxidation procedure, but extremely long reaction times are required to effect substantial oxidation; for practical purposes, then, temperatures above about 120° C. are used. While the composition of the oxidized petroleum waxes so obtained is not fully understood, it is known that they are complex products containing several such oxygenated hydrocarbon materials as

50 acids, hydroxy acids, alcohols, aldehydes, ketones, esters, etc. Oxidized petroleum waxes will be more fully understood from the typical examples provided hereinafter.

The oxidized wax reactants contemplated for use herein are unlike the oxidation products of

many hydrocarbon fractions closely related to those of paraffin waxes and paraffin slackwaxes and, as such, are superior thereto. This superiority carries over in turn to the reaction products of this invention. For example, equal quantities of a paraffin wax, a paraffin slackwax and of hydrocarbon fractions identified in Table 1 below were oxidized by blowing air therethrough at 160-170° C. for approximately the same period of time. The starting materials and oxidation products are described in Table 1 by their neutralization number (N. N.), hydroxyl number and saponification number, each of which is determined by standard procedure known in the art.

Table 1

| Starting Material                                                                 | Reaction Time (Hrs.) | No. of Product | Color        | N. N. | Hydroxyl No. | Saponification No. |
|-----------------------------------------------------------------------------------|----------------------|----------------|--------------|-------|--------------|--------------------|
| Paraffin wax (A. S. T. M. melting point 126° F.)                                  | 31                   | 1              | Light orange | 44    | 36           | 174                |
| Paraffin slackwax                                                                 | 31.5                 | 2              | Dark red     | 8     | 69           | 35                 |
| Hydrocarbon oil (Saybolt Universal Viscosity (S. U. V.) of 60 seconds at 210° F.) | 32                   | 3              | Black        | 2     | 1            | 0                  |
| Hydrocarbon oil (Saybolt Universal Viscosity (S. U. V.) of 55 seconds at 210° F.) | 33                   | 4              | do           | 0.4   | 1            | -2                 |

It will be apparent from the foregoing tabulation that paraffin wax and paraffin slackwax oxidize much more readily than do other typical hydrocarbon fractions, and that the oxidation products of the said waxes are more suitable for the purposes of the present invention in view of their color and oxidation characteristics. In general, it is desirable to carry the oxidation to a point where the hydroxyl and saponification numbers are at least about 20 and the neutralization number is within the range 5 to 60.

As contemplated herein, the amount of  $P_2S_5$  reacted with an oxidized petroleum wax reactant is in the neighborhood of from about 5 per cent to about 15 per cent by weight, with about 10 per cent by weight being preferred.

The reaction temperature used in the preparation of the acidic reaction products defined above is an important consideration. It has been found that elevated temperatures from about 50° C. to about 125° C. are required in order to obtain the desired products, and elevated temperatures of about 100° C. are particularly desirable. If the temperature is too low, as below about 50° C., little or no reaction occurs and if too high, as above about 125° C., undesirable reaction products containing appreciable quantities of oil-insoluble, sludge-like materials are obtained. For example, the reaction product of an oxidized paraffin wax and  $P_2S_5$  at 150° C. is predominantly a black, tar-like, oil-insoluble material.

Illustrative of the reaction products contemplated by the present invention are those shown below in Examples I through IV.

#### EXAMPLE I

A quantity of a paraffin wax having an A. S. T. M. melting point of 126° C. and containing an average of about 24 carbon atoms was oxidized by blowing oxygen therethrough for 31 hours at about 160° C. On analysis, it had an acidity, as measured by its neutralization number (N. N.) of 44, a saponification number of 174 and a hydroxyl number of 36.

A portion of the oxidized paraffin wax (100 parts by weight) was then treated with 10 per cent by weight of  $P_2S_5$  at 100° C. for 3 hours. The reaction mixture thus obtained was filtered and

the filtrate therefrom had an N. N. of 71 and contained 5.06 per cent sulfur and 2.06 per cent phosphorus. This reaction product is identified hereinafter as product A.

#### EXAMPLE II

A quantity of a paraffin slackwax containing about 80 per cent paraffin wax and obtained from a petroleum distillate having a Saybolt Universal Viscosity (S. U. V.) of 120 seconds at 130° F., was oxidized by blowing air therethrough at 160° C. for 31 hours. The oxygenated product was dark red in color and had a neutralization number (N. N.) of 8, a saponification number of 36,

an iodine number of 5 and a hydroxyl number of 69.

(a) A portion of the oxidized paraffin slackwax (100 parts by weight) was reacted with  $P_2S_5$  (10 parts weight) at 100° C. for 2 hours. The reaction product obtained thereby contained 4.9 per cent sulfur and 1.97 per cent phosphorus, and had an N. N. value of 36. This product is referred to herein as product B.

(b) Barium hydroxide octahydrate



(10 parts by weight) was reacted with a quantity of Product B (100 parts by weight) at about 125° C., thereby forming the barium salt of product B. The salt thus obtained—product C—contained 4.36 per cent barium, 4.58 per cent sulfur and 1.44 per cent phosphorus and had an N. N. value of 11.

#### EXAMPLE III

About one per cent (by weight) of the oxidized paraffin wax formed as described in Example I above and having a neutralization number (N. N.) of 40, was added to a paraffin slackwax (identified in Example II) and the resulting mixture was then further oxidized with air at 140° C. for 49 hours. The reaction product thus formed had a neutralization number (N. N.) of 16, a saponification number of 63 and a hydroxyl number of 24.

One hundred parts by weight of the oxygenated paraffin wax so formed was treated with 10 parts by weight of  $P_2S_5$  at 100° C. for 5 hours. The reaction product (product D) contained 4.3 per cent sulfur and 2.06 per cent phosphorus and had a neutralization number (N. N.) of 28.

#### EXAMPLE IV

(a) A quantity (100 parts by weight) of a highly oxidized paraffin wax having a neutralization number (N. N.) of 51, a saponification number of 109 and a hydroxyl number of 56, was reacted with  $P_2S_5$  (10 parts by weight) at 100° C. for 3 hours. The reaction product (product E) contained 5.1 per cent sulfur and 1.12 per cent phosphorus and had a neutralization number (N. N.) of 88.

(b) Ammonia gas was bubbled through a quantity of product E at room temperature (about 20° C.), whereupon the temperature increased several degrees and the product became more viscous. The ammonium salt thus formed contained 2.95 per cent nitrogen, and is referred to herein as product F.

While the acidic reaction products of this invention, such as products A, B, D and E shown above in Examples I through IV, are particularly desirable for use in petroleum fractions (as are the salts of such products), related reaction products prepared in a similar manner from other related hydrocarbon reactants are undesirable for such use. This is demonstrated by the results shown in Table 2 below for products 3 and 4. The oxidized materials shown therein are comparative in that all were prepared in the same manner, as described in connection with Table 1 above. The reaction products shown in Table 2 were prepared by reacting a quantity of an oxidized material (1, 2, 3, and 4, respectively, of Table 1) with  $P_2S_5$  (10 per cent by weight) at 100° C. for the same period of time, about 2 hours.

Table 2

| No. of Product<br>(Table 1) | Color        | N. N. | Hydroxyl<br>No. | Saponification<br>No. | Reaction<br>Product | Color       | N. N. | Percent<br>P | Percent<br>S |
|-----------------------------|--------------|-------|-----------------|-----------------------|---------------------|-------------|-------|--------------|--------------|
| 1                           | Light orange | 44    | 36              | 174                   | A                   | Light brown | 71    | 2.06         | 5.06         |
| 2                           | Dark red     | 8     | 69              | 36                    | B                   | do          | 36    | 1.97         | 4.9          |
| 3                           | Black        | 2     | 1               | 0                     | X                   | Black       | 12    | 0.38         | 0.97         |
| 4                           | do           | 0.4   | 1               | 2                     | Y                   | do          | 7     | 0.27         | 0.86         |

To demonstrate the effectiveness of the reaction products of this invention as mineral oil improving agents, oil blends were prepared containing small quantities of representative reaction products and the blends and the blank oils were subjected to the various tests hereinafter described. It will readily be seen from inspection of the results of these tests that our reaction products are extremely effective in stabilizing mineral oils.

#### CORROSION INHIBITION

Motor oils, especially those refined by certain solvent extraction methods tend to oxidize when submitted to high temperatures and to form products that are corrosive to metal bearings. This corrosive action may be quite severe upon said bearings such as those having the corrosion susceptibility of Cd-Ag alloys and may cause their failure within a comparatively short time. The following test is used to determine the corrosive action of motor oil on an automobile connecting rod bearing.

The oil used consisted of Pennsylvania neutral and residuum stocks separately refined by means of Chlorex and then blended to give an S. A. E. 20 motor oil with a specific gravity of 0.872, a flash point of 435° F. and a Saybolt Universal Viscosity of 318 seconds at 100° F. The oil was tested by adding a section of a bearing containing a Cd-Ag alloy surface, weighing about 6 grams, and heating it to 175° C. for 22 hours while a stream of air was bubbled against the surface of the bearing. The loss in weight of the bearing during this test measures the amount of corrosion that has taken place. A sample of the oil containing a stabilizing agent was run at the same time as a sample of the straight oil, and the loss in weight of the bearing section in the inhibited oil can thus be compared directly.

with the loss of the section in the uninhibited oil. The results are set forth in Table 3 below.

Table 3

| Reaction Product | Conc.<br>Per Cent | Mgms. Loss in<br>Weight |                  |
|------------------|-------------------|-------------------------|------------------|
|                  |                   | Inhib-<br>ited          | Uninhib-<br>ited |
| Product B        | 0.25              | 0                       | .38              |
| Product C        | 0.25              | 1                       | .34              |
| Product D        | 0.25              | 0                       | .32              |
| Product E        | 0.25              | 0                       | .38              |
| Product F        | 0.25              | 0                       | .39              |

#### LAUSON ENGINE TEST

To further demonstrate the effectiveness of the reaction products of this invention as petroleum stabilizing agents a blank oil and blends of the oil and typical reaction products, product C and product D, were subjected to a Lauson engine test. In this test a single cylinder Lauson engine was run with an oil temperature of 290° F. and a jacket temperature of 212° F. The oil was S. A. E. 10 motor oil, solvent refined. The acidity as

Table 4

|                  | N. N. | K. V. @<br>210° F. |
|------------------|-------|--------------------|
| Oil alone        | 10.5  | 9.35               |
| Oil+1% Product C | 0.8   | 5.91               |
| Oil+1% Product D | 0.9   | 5.92               |

#### OXIDATION TEST

A highly refined oil, suitable for use in transformers, had been prepared by treating a coastal distillate with 40 pounds of 98 per cent sulfuric acid and 108 pounds of 103 per cent oleum per barrel, followed by washing and clay percolation. It had a specific gravity of 0.871, a flash point of 310° F. and a Saybolt Universal viscosity of 69 seconds at 100° F. This type of oil tends to form acidic products on oxidation. It was tested by heating samples to 120° C. and bubbling oxygen therethrough for 70 hours. The acids thus formed were determined by treating with alcoholic potash. Results of the oil alone and for the oil plus a reaction product of the type contemplated herein are presented in Table 5 below.

Table 5

|                   | Cone.<br>Per cent | N. N.<br>Value |
|-------------------|-------------------|----------------|
| Oil alone         |                   | 25.0           |
| Oil+0.1 Product C | 0.1               | 0.10           |
| Oil+0.1 Product D | 0.1               | 0.05           |

## RING STICKING AND SLUDGE INHIBITION

That the reaction products contemplated herein are particularly effective in decreasing the tendency of petroleum lubricating oils to cause ring sticking and sludge deposition during the operation of an internal combustion engine is denoted by the results given below in Table 6. This is shown by results of the following test which involves the operation of a single cylinder C. F. R. engine at a speed of 1200 R. P. M. over a time interval of 28 hours. The temperature of the cooling medium of the engine was held at approximately 370° F. and the oil temperature was held at 175° F. during the test. The oil used was a lubricating oil stock of 120 seconds Saybolt Universal viscosity at 210° F. and the conditions observed at the end of the test were: (a) the extent to which the piston rings were stuck, (b) the extent to which the slots in the oil rings were filled with carbonaceous deposits in the oil, and (c) the acidity or neutralization number (N. N.) of the oil. The results obtained from the blank oil and representative blends of the oil and typical reaction products are set forth in Table 6 below.

Table 6

|                  | Ring Conditions, Degrees Stuck |   |     |     |     | Slots, Per cent Filled |    |    | Deposits | N. N. |
|------------------|--------------------------------|---|-----|-----|-----|------------------------|----|----|----------|-------|
|                  | 1                              | 2 | 3   | 4   | 5   | 3                      | 4  | 5  |          |       |
| Oil alone        | 180                            | 0 | 360 | 360 | 360 | 70                     | 90 | 30 | 14.0     | 1.7   |
| Oil+1% Product C | 180                            | 0 | 0   | 0   | 0   | 0                      | 0  | 0  | 5.9      | 1.2   |
| Oil alone        | 360                            | 0 | 360 | 360 | 180 | 60                     | 80 | 40 | 13.8     | 1.6   |
| Oil+1% Product D | 0                              | 0 | 0   | 0   | 0   | 0                      | 0  | 0  | 6.4      | 1.0   |

The results set forth in Tables 3 through 6 above demonstrate that the reaction products contemplated herein prevent the corrosion of hard metal bearings, and inhibit the development of acids and carbonaceous deposits in engines during use. They further indicate that the said reaction products prevent a substantial increase in viscosity of the oil from taking place during such use.

Concentrations of the reaction products contemplated herein from 0.1 per cent to 5 per cent may be used to effect a substantial stabilization of the oil fractions in which they are incorporated. In general, however, from 0.1 per cent to 2.0 per cent will be sufficient. Our reaction products may be used either in straight petroleum fractions or in fractions containing other additives used for other purposes such as detergents, pour point depressants, V. I. improving agents, etc., in which case they serve to stabilize the resulting blend without detracting from the effectiveness of the other additive or additives that may be present.

It is to be understood that while we have hereinabove described typical procedures for making the oil addition agents contemplated herein and have referred to certain specific reaction products and specific mineral oils, the invention is not limited thereto but includes variations of the procedures, and other typical reaction products and petroleum fractions coming within the scope of the appended claims.

We claim:

1. An improved mineral oil composition comprising a major proportion of a viscous mineral oil fraction having in admixture therewith a small amount, sufficient to enhance the stability of said oil fraction, of an oil-soluble, phosphorus- and sulfur-containing material selected from the

group consisting of an acidic reaction product, an ammonium salt thereof and a metal salt thereof, said acidic reaction product being obtained by reaction at a temperature between about 50° C. and about 125° C. of phosphorus pentasulfide and an oxidized paraffin wax characterized by a neutralization number from about 5 to about 60 and hydroxyl and saponification numbers of at least about 20, said oxidized paraffin wax being obtained by oxidizing a paraffin wax having about twenty-four carbon atoms and an A. S. T. M. melting point of 126° F.

2. An improved mineral oil composition comprising a major proportion of a viscous mineral oil fraction having in admixture therewith a small amount, from about 0.1 per cent to about 5.0 per cent, of an oil-soluble, phosphorus- and sulfur-containing material selected from the group consisting of an acidic reaction product, an ammonium salt thereof and a metal salt thereof, said acidic reaction product being obtained by reaction at a temperature between about 50° C. and about 125° C. of phosphorus pentasulfide and an oxidized paraffin wax characterized by a

neutralization number from about 5 to about 60 and hydroxyl and saponification numbers of at least about 20.

3. An improved mineral oil composition comprising a major proportion of a viscous mineral oil fraction having in admixture therewith a small amount, sufficient to enhance the stability of said oil fraction, of an oil-soluble, phosphorus- and sulfur-containing material selected from the group consisting of an acidic reaction product, an ammonium salt thereof and a metal salt thereof, said acidic reaction product being obtained by reaction at a temperature between about 50° C. and about 125° C. of phosphorus pentasulfide and an oxidized paraffin wax characterized by a neutralization number from about 5 to about 60 and hydroxyl and saponification numbers of at least about 20.

4. An improved mineral oil composition comprising a major proportion of a viscous mineral oil fraction, having in admixture therewith a small amount, sufficient to enhance the stability of said oil fraction, of an oil-soluble, acidic, phosphorus- and sulfur-containing reaction product obtained by reaction at a temperature between about 50° C. and about 125° C. of phosphorus pentasulfide and an oxidized paraffin wax characterized by a neutralization number from about 5 to about 60 and hydroxyl and saponification numbers of at least about 20.

5. An improved mineral oil composition comprising a major proportion of a viscous mineral oil fraction having in admixture therewith a small amount, sufficient to enhance the stability of said oil fraction, of an oil-soluble, acidic, phosphorus- and sulfur-containing reaction product obtained by reaction at a temperature between about 50° C. and about 125° C. of phosphorus pentasulfide and an oxidized paraffin wax char-

acterized by a neutralization number from about 5 to about 60 and hydroxyl and saponification numbers of at least about 20, said phosphorus pentasulfide representing from about 5 per cent to about 15 per cent by weight of the said oxidized paraffin wax.

6. An improved mineral oil composition comprising a major proportion of a viscous mineral oil fraction, having in admixture therewith a small amount, sufficient to enhance the stability of said oil fraction, of an oil-soluble, acidic, phosphorus- and sulfur- containing reaction product obtained by reaction at about 100° C. of phosphorus pentasulfide and an oxidized paraffin wax characterized by a neutralization number from about 5 to about 60 and hydroxyl and saponification numbers of at least about 20.

7. An improved mineral oil composition comprising a major proportion of a viscous mineral oil fraction, having in admixture therewith a small amount, sufficient to enhance the stability of said oil fraction, of an oil-soluble, acidic, phosphorus- and sulfur- containing reaction product obtained by reaction at about 100° C. of phosphorus pentasulfide and an oxidized paraffin wax characterized by a neutralization number from about 5 to about 60 and hydroxyl and saponification numbers of at least about 20, said phosphorus pentasulfide representing about 10 per cent by weight of the said oxidized paraffin wax, and the latter being obtained by oxidizing a paraffin wax having about twenty-four carbon atoms and an A. S. T. M. melting point of 126° F.

8. An improved mineral oil composition comprising a major proportion of a viscous mineral oil fraction, having in admixture therewith a small amount, sufficient to enhance the stability of said oil fraction, of an oil-soluble, acidic, phosphorus- and sulfur- containing reaction product obtained by reaction at about 100° C. of phosphorus pentasulfide and an oxidized paraffin slackwax characterized by a neutralization number from about 5 to about 60 and hydroxyl and saponification numbers of at least about 20, said phosphorus pentasulfide representing about 10 per cent by weight of the said oxidized paraffin slackwax, and the latter being obtained by oxidizing a paraffin slackwax containing not less than about 75 per cent of paraffin wax.

9. An improved mineral oil composition comprising a major proportion of a viscous mineral oil fraction, having in admixture therewith a small amount, sufficient to enhance the stability of said oil fraction, of an oil-soluble, acidic, phosphorus- and sulfur- containing reaction product obtained by reaction at about 100° C. of phosphorus pentasulfide and an oxidized paraffin slackwax characterized by a neutralization number from about 5 to about 60 and hydroxyl and saponification numbers of at least about 20, said phosphorus pentasulfide representing about 10 per cent by weight of the said oxidized paraffin slackwax and the said oxidized paraffin slackwax being obtained by oxidizing a paraffin slackwax containing about 80 per cent of paraffin wax.

10. An improved mineral oil composition comprising a major proportion of a viscous mineral oil fraction, having in admixture therewith a

small amount, sufficient to enhance the stability of said oil fraction, of a salt of an oil-soluble, acidic, phosphorus- and sulfur- containing reaction product obtained by reaction at a temperature between about 50° C. and about 125° C. of phosphorus pentasulfide and an oxidized paraffin wax characterized by a neutralization number from about 5 to about 60 and hydroxyl and saponification numbers of at least about 20.

11. An improved mineral oil composition comprising a major proportion of a viscous mineral oil fraction, having in admixture therewith a small amount, sufficient to enhance the stability of said oil fraction, of an ammonium salt of an oil-soluble, acidic, phosphorus- and sulfur- containing reaction product obtained by reaction at about 100° C. of phosphorus pentasulfide and an oxidized paraffin wax characterized by a neutralization number from about 5 to about 60 and hydroxyl and saponification numbers of at least about 20, said phosphorus pentasulfide representing about 10 per cent by weight of said oxidized paraffin wax.

12. An improved mineral oil composition comprising a major proportion of a viscous mineral oil fraction, having in admixture therewith a small amount, sufficient to enhance the stability of said oil fraction, of a metal salt of an oil-soluble, acidic, phosphorus- and sulfur- containing reaction product obtained by reaction at a temperature between about 50° C. and about 125° C. of phosphorus pentasulfide and an oxidized paraffin wax characterized by a neutralization number from about 5 to about 60 and hydroxyl and saponification numbers of at least about 20.

13. An improved mineral oil composition comprising a major proportion of a viscous mineral oil fraction, having in admixture therewith a small amount, sufficient to enhance the stability of said oil fraction, of a barium salt of an oil-soluble, acidic, phosphorus- and sulfur- containing reaction product obtained by reaction at about 100° C. of phosphorus pentasulfide and an oxidized paraffin slackwax characterized by a neutralization number from about 5 to about 60 and hydroxyl and saponification numbers of at least about 20, said phosphorus pentasulfide representing about 10 per cent by weight of said oxidized paraffin slackwax and the said oxidized paraffin slackwax being obtained by oxidizing a paraffin slackwax containing about 80 per cent of paraffin wax.

EVERETT W. FULLER.  
HORACE E. REDMAN.  
HENRY G. BERGER.

#### REFERENCES CITED

The following references are of record in the file of this patent:

#### UNITED STATES PATENTS

| Number    | Name                  | Date          |
|-----------|-----------------------|---------------|
| 2,375,061 | Williams et al. _____ | May 1, 1945   |
| 2,331,923 | Musselman _____       | Oct. 19, 1943 |
| 2,316,088 | Loane _____           | Apr. 6, 1943  |
| 2,281,824 | Bray _____            | May 5, 1942   |
| 2,242,260 | Prutton _____         | May 20, 1941  |